

# UNITED STATES PATENT OFFICE.

ALBERT L. MARSH, OF LAKE BLUFF, ILLINOIS, ASSIGNOR TO THE HOSKINS COMPANY, OF CHICAGO, ILLINOIS, A CORPORATION OF ILLINOIS.

## ELECTRIC RESISTANCE ELEMENT.

No. 853,891.

Specification of Letters Patent.

Patented May 14, 1907.

Application filed January 17, 1907. Serial No. 352,690.

*To all whom it may concern:*

Be it known that I, ALBERT L. MARSH, a citizen of the United States, residing at Lake Bluff, in the county of Lake and State of Illinois, have invented a new and useful Improvement in Electric Resistance Elements, of which the following is a specification.

My object is to provide, as an improved electric resistance material, a metal which has the property of being particularly low in electric conductivity, has a melting-point exceeding that of pure copper, and may be drawn or otherwise shaped to form particularly durable, efficient, and desirable strips, strands, or filaments suitable for use in the various connections where electric resistances are desirable.

I have discovered that the metal vanadium has the properties of being very low in electric conductivity, and very infusible, and that when mixed with nickel or cobalt it forms an alloy having the additional properties of being tough and sufficiently ductile to permit drawing or shaping it into wire or strip form to render it convenient for use as an electric resistance element.

I have found that an alloy consisting of about eighty-five per cent. nickel cobalt and about fifteen per cent. commercially pure vanadium may be drawn into a fine wire and annealed, producing a tough metal having a melting-point exceeding that of pure copper and with an electric resistance approximating fifty times that of pure copper. Its temperature coefficient is particularly low, that of the alloy containing fourteen per cent. of vanadium, being positive about .000345 for each degree C. between 20° and 120°; it does not become crystalline and brittle under heating and cooling; it resists oxidation at ordinary temperature and up to red heat, and it keeps a polish under all atmospheric conditions.

In practice I prefer, mainly for commercial reasons, to form the alloy of preferably less than fifteen per cent. vanadium and more than eighty per cent. nickel. Variations in the relative proportions of the metals affect more or less the variations in strength, durability, and resistivity of the alloy.

It may be stated, for example, that a metal alloy consisting of 14.2 per cent. vanadium and 85.8 per cent. nickel drawn into a wire .40 mm. in diameter has a resistance approximating 3 ohms per foot. The specific resistance of this alloy is about 129 microhms, or more than seventy times the resistance of copper.

While for most purposes alloys of nickel and vanadium containing less than twenty per cent. of vanadium are most practical because of their ductility, all other suitable proportions of these metals are within my invention of the alloy.

In its broadest sense, however, my invention is not limited to an alloy of these metals. Cobalt is suitable for my purpose as the equivalent of nickel; and where I mention in the claims a metal having the properties of nickel and cobalt, I wish to designate only the metals nickel and cobalt which have properties that are the same for my purpose, but which cannot be classed under any single term of which I am aware.

What I claim as new and desire to secure by Letters Patent is—

1. An electric resistance element comprising a strip, strand or filament containing vanadium.
2. An electric resistance element comprising a strip, strand or filament formed of an alloy of vanadium and a metal having the properties of nickel and cobalt.
3. An electric resistance element comprising an annealed strip, strand or filament formed of an alloy of nickel and vanadium.
4. An electric resistance element formed of an alloy consisting of nickel and vanadium.
5. An electric resistance element formed of a metal alloy consisting of vanadium in the proportion of less than twenty per cent. of the element and nickel in the proportion of more than eighty per cent. of the element.

ALBERT L. MARSH.

In the presence of—

J. R. SPENCE,  
C. W. WASHBURN.